

## UNITED STATES PATENT OFFICE

2,070,583

## TEXTILES CONTAINING CELLULOSE DERIVATIVES

William Alexander Dickie and Percy Frederick Combe Sowter, Spondon, near Derby, England, assignors to Celanese Corporation of America, a corporation of Delaware

No Drawing. Application April 26, 1932, Serial No. 607,667. In Great Britain June 18, 1931

14 Claims. (Cl. 28—1)

This invention relates to improvements in materials containing cellulose derivatives and particularly textiles, for instance threads, yarns, fabrics and the like.

As is well known a large number of effects may be obtained, particularly in textile yarns, threads and fabrics, by application of suitable shrinking agents. We have found that methylene chloride, ethylene chloride, chloroform, tetrachlorethane, dichlorethylene, ethyl acetate and like agents are highly satisfactory shrinking agents for cellulose esters and ethers. Not only do the said agents allow of a wide latitude in the amount of shrinkage which takes place, but in addition the materials need not undergo any substantial variation in lustre, if such variation is not desired, and moreover the tensile strength and other valuable properties of the materials are not deleteriously affected. The said agents are not actually solvents for the commercial acetone-soluble cellulose acetate but are capable of swelling the cellulose acetate to a very high degree. When admixed with comparatively small proportions of other agents, and particularly alcohols, which are not themselves solvents for the cellulose acetate, a solvent mixture is produced. The methylene chloride and like agents are customarily termed "latent solvents" for the cellulose acetate and will be so referred to in this specification.

The invention contemplates broadly the application to the materials of methylene chloride, ethylene chloride, dichlorethylene, chloroform, tetrachlorethane, ethyl acetate, or other latent solvents so as to produce a shrinkage effect.

The shrinkage may be utilized to obtain effects of widely varying character in textile yarns, threads or fabrics made of or containing cellulose acetate or other cellulose esters or ethers. Thus, for instance, a cellulose acetate yarn or a yarn made of another cellulose ester or ether may be associated by twisting, knitting or weaving, or any other means with another yarn which is not shrinkable by the methylene chloride or like agent, and the mixed thread or fabric may be treated with the methylene chloride or like agent so as to produce a shrinkage of the cellulose derivative only and thereby produce various effects depending on the character of the material under treatment. In the case of a doubled thread the product resembles to some extent the so-called "slub" yarn. By weaving a fabric with wefts and/or warps alternating with wefts and/or warps of another fibre, the alternation being for example 1:1, 2:2, 2:1 and so forth, pebble, cockle or crêpe effects may be produced. In the case of a weft

of cellulose derivative alternating with another fibre, for example cotton, the warp may consist wholly of cellulose derivative or wholly of another fibre or partly of cellulose derivative and partly of another fibre.

Brocade and like effects may be produced on knitted, woven or other fabrics by the local application of the new shrinking agents to the fabric.

Further the methylene chloride or like shrinking agents of the present invention may be utilized to reduce the tendency of knitted fabrics to ladder, of warp knitted fabrics to split, and of woven fabrics to slip, the shrinking brought about by the agent of the present invention apparently causing a closer packing of the threads, thereby minimizing the tendency to the above faults. Further the invention contemplates the obtainment of any other desired effect by shrinkage, as for example the stretching of umbrella fabrics on their frames by producing a suitable shrinkage.

The methylene chloride or like shrinking agent may be applied by any suitable means depending on the particular effect desired. If it is desired to obtain a uniform treatment, as for example in the treatment of mixed threads, yarns or fabrics or in the preparation of non-laddering, non-splitting or non-slipping fabrics, the agent may be applied for example by a bath treatment, by spraying methods or by padding or in the form of vapour. Local application to obtain brocade or like effects may be achieved by printing methods, for example in conjunction with a suitable thickening agent or by spraying methods, if desired with the use of stencils.

We have found that the shrinking due to the methylene chloride may vary somewhat with the particular type of yarn treated and with its method of preparation, with the concentration of the agent used, with the ester or ether content of the cellulose ester or ether, and of course with the particular cellulose ester or ether. Thus for instance with the ordinary commercial acetone-soluble cellulose acetate the amount of shrinkage achieved with methylene chloride may depend upon the method of preparation of the yarn. We have found that the shrinkage is in general greater with the modern high tenacity wet spun yarns than it is with the commercial dry spun yarns, and moreover with the dry spun yarns is greater if the yarn has been previously subjected to a stretching treatment. Methylene chloride or like agent when used alone produces in general a very high degree of shrinkage, and it is preferable to modify the effect somewhat by the addition of suitable diluents to the methylene chloride or like agent as

for example benzene, toluene, xylene, or other cyclic hydrocarbons, benzine, petrol ether, kerosene and other hydrocarbons of the aliphatic or petroleum series, carbon tetrachloride, trichloroethylene, perchlorethylene and other chlorinated or halogenated compounds which are inert or comparatively inert towards the cellulose derivative. Alcohols may be employed as diluents, though of course they will be used in proportions which with the methylene chloride or like agent does not constitute a solvent mixture. However, we prefer diluents which are not miscible with water. We find it preferable to restrain the high shrinking action of the methylene chloride or like agent by the addition of such a diluent so as to reduce the concentration of the methylene chloride to about 60 to 70%. Benzene and carbon tetrachloride are very suitable diluents for use with methylene chloride in such a concentration. In some cases a powerful latent solvent such as methylene chloride may be diluted with a less powerful latent solvent such as dichlorethylene. Thus for instance mixtures containing 70-80% of dichlorethylene and 30-20% of methylene chloride yield very good results. If desired the amount of shrinkage may be modified by exerting a suitable tension upon the yarn, thread or fabric under treatment, such tension being either insufficient to prevent some shrinkage or being sufficient to prevent shrinkage, the tension being subsequently decreased or removed so as to enable the shrinkage to take place.

The present invention further includes the production of shrinkage effects by means of a differential shrinkage obtainable as described above between two or more different types of cellulose derivative yarn, for example wet and dry spun yarns or yarns of different esters or ethers or of different ester or ether content. Such differentially shrinkable yarns may be used alone or in conjunction with other fibres.

Of the various fibres which may be used in association with the shrinkable cellulose derivative yarns and which are substantially unshrinkable by the methylene chloride or like agents, mention may be made of natural silk, wool, cotton and the cellulosic type of artificial silk.

While the invention has been described above more particularly with reference to materials composed of or containing acetone-soluble cellulose acetate, it may be applied to materials made from or containing other cellulose acetates or other esters, for example cellulose formate, propionate, butyrate, nitro acetate and the like, or made from or containing cellulose ethers, for instance methyl, ethyl or benzyl cellulose or made from or containing cellulose ether-esters.

What we claim and desire to secure by Letters Patent is:—

1. Process for the production of shrinkage effects on artificial materials containing filaments, threads, yarns and the like of organic derivatives of cellulose having at most only a low degree of twist, which comprises applying to said materials, in the presence of a water-immiscible diluent, a swelling agent which is a latent solvent for the cellulose derivative, and allowing the materials to shrink.

2. Process for the production of shrinkage effects on filaments, threads, yarns and like materials containing organic derivatives of cellulose and having at most only a low degree of twist and on fabrics containing the same, which comprises applying thereto, in the presence of a water-immiscible diluent, a halogenated hydrocarbon

swelling agent which is a latent solvent for the cellulose derivative, and allowing the materials to shrink.

3. Process for the production of shrinkage effects on filaments, threads, yarns and like materials containing acetone-soluble cellulose acetate and having at most only a low degree of twist and on fabrics containing the same, which comprises applying thereto methylene chloride, in the presence of a diluent which is not miscible with water, and allowing the materials to shrink.

4. Process for the production of shrinkage effects on filaments, threads, yarns and like materials containing organic derivatives of cellulose and having at most only a low degree of twist and on fabrics containing the same, which comprises locally applying thereto a swelling agent which is a latent solvent for the cellulose derivative and which is dissolved in a water-immiscible diluent, and allowing the materials to shrink.

5. Process for the production of shrinkage effects on filaments, threads, yarns and like materials containing organic derivatives of cellulose and having at most only a low degree of twist and on fabrics containing the same, which comprises locally applying thereto, in the presence of a water-immiscible diluent, a halogenated hydrocarbon swelling agent which is a latent solvent for the cellulose derivative, and allowing the materials to shrink.

6. Process for the production of shrinkage effects on filaments, threads, yarns and like materials containing acetone-soluble cellulose acetate and having at most only a low degree of twist and on fabrics containing the same, which comprises locally applying thereto methylene chloride in presence of a diluent which is not miscible with water, and allowing the materials to shrink.

7. Process for the production of shrinkage effects on mixed threads or yarns having at most only a low degree of twist and mixed fabrics and like materials composed of yarns having at most only a low degree of twist and containing at least one organic derivative of cellulose, which comprises shrinking in selected areas with a swelling agent which is a latent solvent for the organic derivative of cellulose and which is dissolved in a water-immiscible diluent, materials containing constituents having different reactions to the shrinking action of said latent solvent.

8. Process for the production of shrinkage effects on mixed threads or yarns having at most only a low degree of twist and mixed fabrics and like materials composed of yarns having at most only a low degree of twist and containing at least one organic derivative of cellulose, which comprises shrinking in selected areas, in the presence of a diluent not miscible with water, with a halogenated hydrocarbon swelling agent which is a latent solvent for the organic derivative of cellulose, materials containing constituents having different reactions to the shrinking action of said latent solvent.

9. Process for the production of shrinkage effects on mixed threads or yarns having at most only a low degree of twist and mixed fabrics and like materials composed of yarns having at most only a low degree of twist and containing organic derivatives of cellulose, which comprises shrinking with a swelling agent which is a latent solvent for the organic derivatives of cellulose and which is dissolved in a water-immiscible diluent, materials containing organic derivatives of cellulose having different reactions to the shrinking action of said latent solvent.

10. Process for the production of shrinkage

- effects on mixed threads or yarns having at most only a low degree of twist and mixed fabrics and like materials composed of yarns having at most only a low degree of twist and containing at least 5 one organic derivative of cellulose, which comprises shrinking in the presence of a water-immiscible diluent and with a halogenated hydrocarbon swelling agent which is a latent solvent for the organic derivative of cellulose, materials 10 containing constituents having different reactions to the shrinking action of said latent solvent.
11. Process for the production of shrinkage effects on mixed threads or yarns having at most only a low degree of twist and mixed fabrics and like materials composed of yarns having at most 15 only a low degree of twist and containing at least one organic derivative of cellulose, which comprises shrinking with methylene chloride in the presence of a diluent which is not miscible with water, materials containing constituents having different reactions to the shrinking action of methylene chloride.
12. Process for the production of shrinkage effects on mixed threads or yarns having at most only a low degree of twist and mixed fabrics and like materials composed of yarns having at the most only a low degree of twist and containing at least 20 an acetone-soluble cellulose acetate, which comprises shrinking with a swelling agent which

is a latent solvent for the cellulose acetate and which is dissolved in a water-immiscible diluent, materials containing constituents having different reactions to the shrinking action of said latent solvent. 5

13. Process for the production of shrinkage effects on mixed threads or yarns having at the most only a low degree of twist and mixed fabrics and like materials composed of yarns having at the most only a low degree of twist and containing 10 at least an acetone-soluble cellulose acetate, which comprises shrinking, in the presence of a diluent not miscible with water and with a halogenated hydrocarbon swelling agent which is a latent solvent for the cellulose acetate, materials containing constituents having different reactions to the shrinking action of said latent solvent. 15

14. Process for the production of shrinkage effects on mixed threads or yarns having at the most only a low degree of twist and mixed fabrics 20 and like materials composed of yarns having at the most only a low degree of twist and containing at least an acetone-soluble cellulose acetate, which comprises shrinking with a 60 to 70% solution of methylene chloride in benzene, materials 25 containing constituents having different reactions to the shrinking action of such reagent.

WILLIAM ALEXANDER DICKIE.  
PERCY FREDERICK COMBE SOWTER.